

## UNITED STATES PATENT OFFICE

GEORGE A. RICHTER AND WALLACE B. VAN ARSDEL, OF BERLIN, NEW HAMPSHIRE,  
ASSIGNORS TO BROWN COMPANY, OF BERLIN, NEW HAMPSHIRE, A CORPORATION OF  
MAINE

## ARTIFICIAL LEATHER FABRICATION

No Drawing.

Application filed September 27, 1929. Serial No. 395,744.

This invention deals with the fabrication of artificial leather, its object being to produce a product which, while useful in various fields, as in making upholstered furniture, automobile tops, travelling bags, and the like, is more particularly designed for use in making shoe parts, such as inner soles.

Artificial leather shoe parts, in order to be acceptable by the trade, must have characteristics closely resembling the natural product. For example, an artificial leather innersole should have high flexibility, tensile strength, and tear resistance, and should be resilient and of sufficient porosity to permit breathing of the foot and to absorb perspiration therefrom. It has been found that a satisfactory article may be obtained by impregnating a foundation of loosely felted cellulose fiber with a rubber-carrying liquid vehicle such as so-called rubber solutions in organic solvents or aqueous dispersions of rubber, and then removing the liquid vehicle, and if desired, vulcanizing the rubber-impregnated product. Upon the removal of the liquid vehicle, the rubber serves to bind together the fibers of the foundation and sufficient porosity is restored thereto so that it is capable of readily absorbing moisture. When a highly porous web of loosely felted cellulose fiber is used as a foundation and the dried, rubber-impregnated product contains about 90% to 110% rubber solids, based on the weight of dry fiber, it has been found that the product has the all-round characteristics sought for in articles such as innersoles. It is sometimes desired to coat the innersole with materials such as lacquers, in order to obtain such qualities as gloss and smoothness to the foot.

If an innersole of the type hereinbefore described is coated with a lacquer, considerable porosity and resiliency is lost, since the lacquer penetrates into and fills the pores of the sole. We have observed that a comparatively small change in the rubber content of such soles is associated with an unexpectedly great change in characteristics such as tensile strength, tear resistance, and porosity. For instance, a sole having a rubber content of about 70%, based on the weight of dry fiber, is notably inferior in strength

to a similar sole having a rubber content of about 110%, but we have further observed that the sole of lower rubber content may be coated with material such as lacquers without becoming so lacking in porosity and resiliency as the sole of higher rubber content.

In accordance with the present invention, we produce a rubber-impregnated sheet of interfelted cellulose fibers, a surface portion of which is of lower rubber content than the rest of the sheet, so that when the surface of this portion is coated or dressed with materials such as lacquers, undesirable change in characteristics such as porosity and resiliency will be minimized, and the resulting product will have the desired high strength and at the same time be free from the objectionable rubbery feel experienced when the surface portion contains a large amount of rubber. In making an artificial leather suitable for use in making shoe parts such as innersoles, this may be accomplished by bonding together one or more porous, rubber-impregnated webs with another porous, rubber-impregnated web having lower rubber content and higher porosity as the surface ply, the surface of the latter ply being coated with a material such as a lacquer. While it is not absolutely necessary, it is preferable to coat the surface ply and to emboss it before it is united to the rest of the material. This is especially the case if any embossing is done because the high pressure of an embossing press would tend to produce a very high density and uncertain thickness in the entire sole. The outer ply or plies of the soles may have a rubber content of, say, about 90% to 110%, and the inner or surface ply a rubber content of about 70% to 90%, based on the weight of dry fiber.

A procedure which may be followed in producing the product of the present invention, may be substantially as follows. A fluffy web composed of loosely interfelted cellulose fibers and possessing high porosity is preferably used as the foundation for all the plies. A web of unusually high porosity may be produced by using a substantially unbeaten wood fiber of high alpha cellulose content, say, 94% or greater, as a raw material, and

forming such fiber into a web on a paper-making machine designed to effect dewatering and drying of the web without the application of the heavy pressures used in ordinary papermaking practice. While other fibers in substantially unbeaten condition, such as sulphite, kraft, or soda pulp, may be employed, a substantially unbeaten wood fiber of high alpha cellulose content is preferred, because it is more highly absorptive than the usual unbeaten commercial wood fibers, and hence enhances the absorptivity or porosity resulting from the loosely felted, uncompacted condition of the fibers. The dry, porous web may be passed through a bath of rubber-carrying vehicle such as an ammonia-preserved latex diluted to a solids content of, say, about 16%, at which content immersion for about five to thirty seconds effects a thorough impregnation of the web. If to be used as the outer plies of the sole, the impregnated web may be squeezed until its rubber solids content is about 110%, based on the weight of dry fiber, and if to be used as the inner or surface plies, until its rubber solids content is about 70%. The rubber content of the inner plies may be reduced not only by squeezing them harder but also by diluting the latex further, say, to 14% instead of 16% solids content. In order to prevent migration of the rubber globules to the surface of the web during drying, the ammonia-preserved latex may be treated with the oxide of an amphoteric metal, preferably zinc oxide, as described in application Serial No. 369,267, filed June 7, 1929, by Roger B. Hill, or with alkaline earth metal hydroxides, preferably slaked lime, as described in application Serial No. 373,055, filed June 22, 1929, by Roger B. Hill. When slaked lime is the compound added to the latex to overcome migration tendencies during drying, protective colloids such as soluble soaps or caseinates which are capable of being precipitated by lime as insoluble calcium soaps or caseinates, are preferably added to the latex prior to the addition of the slaked lime in order to overcome coagulating tendencies. Such treatment of the latex prior to its use for the impregnation of the web makes possible the production of a dried, rubber-impregnated web of uniformity in respect of rubber distribution therethrough, as troublesome non-rubber constituents of the latex, namely, the proteins and the resins, are converted to an insoluble, inert condition. Apparently, setting or coagulation of the rubber by drying is so retarded by the proteins and resins which exist respectively in an ammonia-preserved latex as water-soluble proteinates and alkali resinates, that there is a tendency for rubber particles to migrate to the surface of the impregnated product, where evaporation of water is taking place. The tendency for migration of rubber particles is especially pronounced in the case of

highly porous webs of cellulose fiber of the type described, evidently because of the high capillary action taking place during drying to cause such migration. When such compounding agents as lime and casein are used, the ratio of total impregnating solids to fiber may with advantage be raised from, say, 110% to 115%, or even to 200%, based on dry fiber. In such a case, however, the actual ratio of rubber to fiber would still not be much above 110%, since a composition as low in rubber content as 60% may be used.<sup>70</sup><sup>75</sup>

If desired, a vulcanized latex may be used, so that when the latex-impregnated web is subsequently dried, the rubber will be coagulated in the web in vulcanized condition. Or artificial aqueous dispersions may be used in lieu of natural latex. Suitable rubber-compounding materials, vulcanizing agents, and accelerators of vulcanization may be added to the artificial or natural rubber dispersion, so that the dried, rubber-impregnated web may be vulcanized under the action of heat, if desired.<sup>80</sup><sup>85</sup>

The web used as a foundation material is preferably comparatively thin, so that it may be impregnated rapidly and uniformly. In actual practice, a web of about 100 pounds basis weight (i. e., the weight of 2880 sq. ft. of web) may be employed to good advantage. The impregnated web is of insufficient thickness for the manufacture of products such as innersoles, it being necessary to bond together two or more sheets. One or more sheets impregnated to a rubber content of about 110%, and a sheet impregnated to a rubber content of about 90% may be bonded together by latex, the sheet of lower rubber content constituting a surface ply of the resulting product. It has been found advantageous to moisten or wet the surfaces of the dried, rubber-impregnated sheets and then to apply a comparatively thick or concentrated latex as the bonding material, whereupon the sheets may be superposed, united under pressure, and dried. Apparently, the initial moistening or wetting of the plies promotes penetration of the thick latex into the surface portion of the plies and results in a better interlocking of the plies after the latex is dried.<sup>90</sup><sup>100</sup><sup>105</sup><sup>110</sup><sup>115</sup>

The inner ply may be surfaced with a suitable coating material, a nitrocellulose lacquer being preferable, because it imparts desirable gloss and smoothness to the foot, and is permanent against the action of perspiration. Nitrocellulose lacquer, while preferable, is not by any means the only finish which may be used. Other finishes such as are used on kid and sheep skins may be applied where gloss and color are much more important than permanence. The lacquer may be applied as by spraying, whereupon the coated product may be dried. If desired, the lacquered surface may be em-<sup>120</sup><sup>125</sup><sup>130</sup>

bossed, preferably before uniting with the other plies, to produce grain effects simulating those of natural leather.

The surface treatment may include steps in addition to those hereinbefore given. For instance, an initial or base coat of clear nitrocellulose lacquer may be applied to the surface of the sheet, whereupon one or more coats of nitrocellulose lacquer containing suitable pigments or fillers may be applied. The base coat prevents sinking of the pigments or fillers into the rubber-impregnated foundation, where they are undesirable. The lacquered and pigmented surface may then be embossed and a final coat of clear nitrocellulose lacquer may be applied thereto. The lacquered surface may then be smooth-plated to destroy the oily or greasy appearance and to bring out the gloss. The finished product may then be united with the other plies and cut into innersoles or used in making other articles where artificial leather having the characteristics of such a product is desired.

We claim:

1. An artificial leather comprising a rubber-impregnated sheet of interfelted cellulose fibers having a surface portion of lower rubber content than the rest of the sheet.

2. An artificial leather comprising a rubber-impregnated sheet of interfelted cellulose fibers having a surface portion of lower rubber content than the rest of the sheet and surfaced at said portion with a coating material.

3. An innersole comprising a plurality of superposed, rubber-impregnated plies of interfelted cellulose fibers, the rubber content of the inner ply being lower than the rubber content of the other plies.

4. An innersole comprising a plurality of superposed, rubber-impregnated plies of interfelted cellulose fibers bonded together with rubber, the rubber content of the inner ply being lower than the rubber content of the other plies, said inner ply being surfaced with a coating material.

5. An innersole comprising a plurality of superposed, rubber-impregnated plies of interfelted cellulose fibers bonded together with rubber, the solids content including rubber of the inner ply being about 70% to 90%, based on the weight of dry fiber and the solids content including rubber throughout the other plies being about 110% to 200%, said inner ply being surfaced with nitrocellulose lacquer and embossed to the desired grain-effect.

6. A method which comprises superposing and bonding together a plurality of rubber-impregnated webs of interfelted cellulose fibers of different rubber contents with the web of low rubber content as an outer ply and the surface of which outer ply is finished with a coating material.

7. A method which comprises impregnating a plurality of webs of cellulose fibers with a rubber-carrying liquid vehicle to different rubber contents, removing the liquid vehicle, applying lacquer to the surface of the ply of low rubber content, embossing the lacquered surface to the desired grain effect, superposing and uniting it as a surface ply with the other rubber-impregnated webs, and cutting into innersoles.

8. An artificial leather comprising a rubber-impregnated, loosely interfelted, paper machine-made foundation of wood fibers of high alpha-cellulose content having a surface portion of lower rubber content than the rest of the foundation.

In testimony whereof we have affixed our signatures.

GEORGE A. RICHTER.  
WALLACE B. VAN ARSDEL.

85

90

95

100

105

110

115

120

125

130